

Nov. 17, 1964

R. P. DURHAM

3,157,585

CHROMIUM PLATING

Filed Dec. 18, 1959



INVENTOR.  
Rolle P. Durham  
BY  
S. N. Shampo  
ATTORNEY

1

3,157,585

## CHROMIUM PLATING

Rollie P. Durham, Flint, Mich., assignor to General Motors Corporation, Detroit, Mich., a corporation of Delaware

Filed Dec. 18, 1959, Ser. No. 860,436  
5 Claims. (Cl. 204—41)

This invention relates to electroplating and more particularly to chromium plated articles of exceptional durability and to a method of forming such articles.

The present disclosure is a continuation-in-part of my co-pending United States patent application Serial No. 812,081, which was filed on May 11, 1959, and assigned to the assignee of the instant patent application.

Since the initial use of chromium in decorative plating, the problem of obtaining decorative coatings of satisfactory durability has been a problem. Moreover, for unknown reasons the quality of a chromium coating will vary from time to time even though the coatings are deposited from the same solution apparently under exactly the same conditions.

Accordingly, it is a primary purpose of this invention to provide decorative chromium plated parts which exhibit vastly improved durability and to provide a method of forming such articles with an unusual degree of consistency.

In general my invention involves forming decorative chromium plated parts by applying at least two chromium layers of different characteristics to a suitably prepared surface of a part. A careful selection of the individual layers used in accordance with the invention permits the consistent formation of chromium plated parts which are not only more durable than conventional chromium coatings but also permit chromium plated steel parts to be produced which do not fail to red rust under comparatively severe corrosion testing.

The preparation of the part prior to applying my chromium coating is as important to my invention as it is to conventional chromium plating. Accordingly best durability has been obtained when protective surface coatings interjacent the chromium coating and the surface of the metal part are used. For example, I prefer to apply the dual layer film to a steel part which has been coated successively with copper and nickel in the known and accepted manner of preparing steel parts for chromium plating.

As a specific example of the practice of my invention a metal part, such as one made from SAE 1010 steel, is polished and cleaned to form a suitable surface for subsequently applied electrodeposited coatings. The particular manner in which the metal part is cleaned is only as material to my invention as it is to any general electroplating procedure and may, therefore, be varied considerably.

In one method of cleaning, the workpiece is anodically treated in an alkaline solution which is made up as follows:

Oz./gal.

|                           |   |
|---------------------------|---|
| Sodium orthosilicate      | 8 |
| Tetrasodium pyrophosphate | 1 |
| Sodium carbonate          | 1 |

Using a bath temperature of approximately 160° F. to 180° F. the workpiece is subjected to an anodic potential for 60 seconds to 70 seconds with a current density of approximately 50 amperes per square foot to 100 amperes per square foot.

After the anodic cleaning the part is then thoroughly rinsed in cold water and then immersed for approximately 40 seconds in a room temperature aqueous bath containing 25% muriatic acid, by volume.

2

Subsequently the part is removed from the muriatic acid bath and thoroughly rinsed. The part is then anodically cleaned a second time in the manner described above but only for approximately 30 seconds. It is then removed from the anodic cleaning bath and again rinsed and immersed for about 10 seconds in the muriatic acid bath and then thoroughly rinsed.

After cleaning, the workpiece is preferably immersed in a copper or nickel strike solution to insure good adherence of subsequently electrodeposited coatings. One such solution which can be employed to apply a thin coating of copper to the part contains the following ingredients:

|                       | Oz./gal. |
|-----------------------|----------|
| 15 Copper cyanide     | 2-4      |
| Sodium cyanide (free) | 1.5-2    |
| Caustic soda          | 2-3      |

A negative potential is applied to the part for a sufficient duration, approximately 170 seconds, under a cathode current density of approximately 20 amperes per square foot to 25 amperes per square foot in order to apply about .0001 inch of copper.

The part is subsequently removed from the copper strike bath, rinsed and then dipped in a dilute aqueous solution of sulfuric acid, 5%  $H_2SO_4$  by volume. Immersion for about 10 seconds in this bath, which is at room temperature, aids in keeping the copper surface active to improve adhesion of the subsequently applied thicker copper coating. The part is then removed from the sulfuric acid bath, rinsed and immersed in an acid copper plating solution. A suitable acid copper bath has a composition as follows:

|                              |          |          |
|------------------------------|----------|----------|
| 35 Cupric sulfate (hydrate)  | oz./gal. | 22-26    |
| Sulfuric acid (concentrated) | oz./gal. | 8        |
| Thiourea                     | oz./gal. | 0.000589 |
| Sodium lauryl sulfate        | oz./gal. | 0.00566  |
| Molasses                     | ml./l.   | .25      |

With air and cathode rod agitation, direct electric current is passed through the solution and copper anodes so as to impose a negative potential on the workpiece for a sufficient duration to deposit a copper coating of at least about 0.0015 inch. The bath is preferably maintained at a temperature of approximately 70° F. to 90° F. while the cathode current density is maintained at approximately 50 amperes per square foot.

Although in some instances the workpiece can be nickel plated directly after removal, most generally it is preferred to buff the copper coating bath prior to immersion in a nickel plating solution. After buffing, of course, the workpiece must be cleaned again to prepare the copper surface for reception of the nickel plate.

As the initial cleaning, this latter cleaning can be accomplished satisfactorily in the normal and accepted manner for such cleaning, such as by a cathodic electrolysis, an anodic electrolysis, and an acid dip. Thus, after buffing the part is electrolyzed for 30 seconds to 60 seconds in an aqueous bath having about 2 ounces per gallon to 6 ounces per gallon of a mixture containing, by weight, about 55% soda ash, 25% trisodium orthophosphate and 20% caustic soda. Using a bath temperature of about 160° F., a negative potential is imposed on the workpiece sufficient to cause a cathode current density of about 50 amperes per square foot.

The part is then anodically cleaned in the manner described above for about 30 seconds, rinsed and then dipped in a dilute, sulfuric acid solution (1%  $H_2SO_4$ , by volume, in water) for 20 second to 30 seconds.

After immersion in the dilute acid solution, the part was thoroughly rinsed and immersed in a bright nickel

electroplating tank. One such solution which is suitable for depositing bright metal has the following ingredients:

|                                  |         |         |
|----------------------------------|---------|---------|
| Nickel sulfate (hydrated) -----  | oz./gal | 30-50   |
| Nickel chloride (hydrated) ----- | oz./gal | 4-10    |
| Boric acid -----                 | oz./gal | 5-8     |
| Wetting agent -----              | oz./gal | 0.00566 |
| Primary brightener -----         | g./l.   | 2-5     |
| Secondary brightener -----       | mg./l.  | 2-100   |

Direct electric current is passed through the solution with cathode rod agitation so as to impose a negative potential on the part for a sufficient duration to deposit a nickel coating of at least about 0.0005 inch. The bath is preferably maintained at a temperature of approximately 120° F. to 150° F. and the cathode current density is maintained at approximately 40 amperes per square foot to 60 amperes per square foot.

When a sufficient thickness of nickel has been deposited on the part, it is removed from the nickel electroplating bath, rinsed and placed in contact with a suitable chromium plating solution.

With the preliminary copper and nickel layers applied, a plurality of chromium layers is then deposited thereover. The use of a plurality of chromium layers to improve durability of a decorative chromium plated part is known in the art. However, the plurality of layers applied by prior procedures does not present the material improvements in durability such as are obtainable with my invention. I have found that remarkable increases in durability of the part are obtained when the part is coated with a plurality of chromium coatings having different characteristics.

It is well known that chromium layers deposited from different bath compositions and even from the same bath under different conditions may have distinctly different characteristics. I have found that some combinations of chromium layers having certain characteristics will produce a remarkably unexpected improvement in corrosion resistance not obtainable by other combinations of chromium layers. For example, I have found that the marked increases in corrosion resistance can be obtained in a dual layer chromium coating if the first layer (Layer A) is electrodeposited from a sulfate catalyzed chromium plating bath, and the second or outermost layer (Layer B) is electrodeposited from an aqueous bath formed in accordance with United States Patent No. 2,640,022, Stareck. The following Baths I and II will serve as specific examples, respectively, of suitable baths for electrodepositing Layers A and B:

*Bath I*

Oz./gal.

|                                      |    |
|--------------------------------------|----|
| CrO <sub>3</sub> -----               | 40 |
| H <sub>2</sub> SO <sub>4</sub> ----- | 40 |

*Bath II*

26.0

|                                                     |      |
|-----------------------------------------------------|------|
| CrO <sub>3</sub> -----                              | 26.0 |
| K <sub>2</sub> Cr <sub>2</sub> O <sub>7</sub> ----- | 4.9  |
| SrCrO <sub>4</sub> -----                            | 0.6  |
| K <sub>2</sub> SiF <sub>6</sub> -----               | 1.4  |
| SrSO <sub>4</sub> -----                             | 0.8  |

The initial chromium layer (Layer A) is deposited from Bath I under a cathode current density of approximately 140 amperes per square foot at a bath temperature of approximately 120° F. for approximately 5 minutes to 6 minutes to produce a minimum coating thickness of at least 0.000015 inch. The part is then thoroughly rinsed and directly passed into Bath II which is maintained at a temperature of approximately 120° F. The bath is electrolyzed at a cathode current density of approximately 125 amperes per square foot for a sufficient duration to obtain a minimum coating thickness of about 0.000015 inch.

Although optimum results are obtained by applying Layer A in the manner indicated above, improvements can be obtained using any of the bath formulations and conditions which are generally satisfactory for applying

single coatings of chromium from a sulfate catalyzed bath. Generally Layer A can be formed in the normal and accepted manner of electrodepositing chromium from a sulfate catalyzed bath. In most instances highly satisfactory results are obtained with my invention if Layer A is deposited from the sulfate catalyzed bath in the manner which would provide best durability if Layer A were used as a single layer. The chromium coating of this example of my invention generally provides optimum results if Layer A is deposited with as sparse a crack pattern as possible.

Similarly, the composition of Bath II, as well as the conditions of using it, can be varied. The composition of Bath II and its conditions of use can vary generally as described in United States Patent No. 2,640,022, Stareck. These variations are as material to the subject invention as they are to conventional chromium plating to obtain maximum durability. In most instances optimum results are obtained when Layer B is deposited so as to have a relatively dense crack pattern when compared to Layer A.

It has also been found that the advantages of my invention can also be obtained using a bath composition made up in accordance with the aforementioned United States Patent No. 2,640,022, Stareck, hereinafter listed as Bath IV, in conjunction with a bath composition and method of chromium plating such as described in United States Patent No. 2,916,424, Stareck et al., hereinafter listed as Bath III. The immediately following disclosure of Baths III and IV and the method of using same is presented to serve as a specific example of this embodiment of the invention.

*Bath III*

G./l.

|                                                     |      |
|-----------------------------------------------------|------|
| CrO <sub>3</sub> -----                              | 400  |
| SO <sub>4</sub> ion -----                           | 1.66 |
| SiF <sub>6</sub> ion -----                          | 1.66 |
| K <sub>2</sub> Cr <sub>2</sub> O <sub>7</sub> ----- | 3.5  |

*Bath IV*

Oz./gal.

|                                                     |     |
|-----------------------------------------------------|-----|
| CrO <sub>3</sub> -----                              | 40  |
| K <sub>2</sub> Cr <sub>2</sub> O <sub>7</sub> ----- | 4.9 |
| SrCrO <sub>4</sub> -----                            | 0.6 |
| K <sub>2</sub> SiF <sub>6</sub> -----               | 1.6 |
| SrSO <sub>4</sub> -----                             | 0.8 |

The initial chromium layer (Layer A) is deposited from Bath III under a cathode current density of approximately 220 amperes per square foot at a bath temperature of approximately 120° F. for a sufficient duration to produce a minimum coating thickness of about 0.000015 inch. The bath was then thoroughly rinsed and directly passed into Bath IV which was maintained at a temperature of approximately 120° F. Bath IV was then electrolyzed at a cathode current density of approximately 200 amperes per square foot for a sufficient duration to obtain a minimum coating thickness of approximately 0.000015 inch.

The sulfate ion concentration in Bath III was attained by adding suitable amounts of sulfuric acid to the bath solution which was previously saturated with strontium sulfate. The silicofluoride ion concentration was attained using K<sub>2</sub>SiF<sub>6</sub>.

The aforementioned United States Patent No. 2,916,424, Stareck et al., is specifically directed to providing a process for plating crack-free chromium surfaces of mirror-brightness to a thickness of at least 0.00005 inch. However, it has been found that unexpectedly improved durability of chromium plated parts can be attained with the process described in the above-mentioned Stareck et al. patent, when used in my invention, even if it is modified by depositing a lesser thickness of chromium. As indicated above, significantly improved results have been obtained when the deposit of the Layer A chromium is only about 0.000015 inch in thickness.

The aforementioned United States Patent No. 2,916,424, Stareck et al., discloses a relationship pertinent to Bath III between temperature, concentration and ratio, such as illustrated by FIGURES 1 and 2. The sulfate and silicofluoride ions in Bath III are referred to as catalyst ions. The term "ratio" as used in the discussion of FIGURES 1 and 2 refers to the ratio of the weight of  $\text{CrO}_3$  to the weight of the catalyst ions in the bath.

Stareck et al. disclose that bright, crack-free chromium can be electroplated at temperatures between 112° F. and 119° F. as shown in FIGURE 1 by using a high ratio. FIGURE 1 also indicates that at 115° F. a ratio of about 115:1 is the limiting ratio whereas at 112° F. it is 150:1. It is further stated that in many combinations of the three variables; temperature, concentration and ratio, electrodeposition of bright, crack-free chromium between the temperatures of 117° F. and 135° F. is preferred. It is preferred to utilize  $\text{CrO}_3$  concentrations between about 250 grams per liter and about 425 grams per liter within this latter temperature range; the relationship between the three variables being defined by the areas enclosed by the curve in FIGURE 2. Within the enclosed area ABC in FIGURE 2, ratios of 80:1 and 150:1 may be used. Within the area defined as ABD, the preferred range of ratios is narrower with the limiting preferred range at the line ADB being 115:1 to 150:1.

It is further stated that bright, crack-free chromium can be deposited at a maximum thickness when plating with the rectangular area ABCD of FIGURE 1 at ratios between about 105:1 to 135:1, wherein baths having a  $\text{CrO}_3$  concentration between about 275 grams per liter and 400 grams per liter and plating temperatures of about 125° F. and 138° F. are used.

When the temperatures and the  $\text{CrO}_3$  concentrations are maintained within the area defined by the closed curve ADFG in FIGURE 1, it is stated as possible to deposit bright, crack-free chromium in all ratios between 80:1 and 150:1.

The advantages of the invention have also been obtained by applying a chromium coating having a plurality of alternately different chromium layers using two sulfate catalyzed chromium plating baths having compositions as follows:

*Bath V*

|               | Oz./gal. |
|---------------|----------|
| Chromic acid  | 26       |
| Sulfuric acid | .26      |

*Bath VI*

|               |     |
|---------------|-----|
| Chromic acid  | 40  |
| Sulfuric acid | .40 |

The initial chromium layer (Layer A) was deposited from Bath V, which was at a temperature of approximately 102° F. to 106° F., under a cathode current density of approximately 108 amperes per square foot. The bath was electrolyzed for approximately 7½ minutes to apply a minimum coating thickness of about 0.000015 inch. The part was then removed from Bath V, thoroughly rinsed and placed in Bath VI, which was at a temperature of approximately 122° F. to 126° F. The second layer (Layer B) was deposited from Bath VI under a cathode current density of 144 amperes per square foot for approximately 5 minutes to obtain the minimum Layer B thickness of about 0.000015 inch.

Layer A should be deposited with a relatively sparse crack pattern while Layer B should be deposited with a comparatively dense crack pattern. Baths V and VI can be varied to some extent without losing the benefits of the invention. For example Layer A and Layer B can,

respectively, be satisfactorily formed using bath compositions and conditions such as follows:

*Bath V(A)*

|   |                                 |                      |
|---|---------------------------------|----------------------|
| 5 | Chromic acid                    | 20-35 oz./gal.       |
|   | Sulfuric acid                   | .20-.35 oz./gal.     |
|   | Temperature                     | 95° F.-115° F.       |
|   | Average cathode current density | 90 a.s.f.-140 a.s.f. |

*Bath VI(A)*

|    |                                 |                       |
|----|---------------------------------|-----------------------|
| 10 | Chromic acid                    | 40-70 oz./gal.        |
|    | Sulfuric acid                   | .45-.70 oz./gal.      |
|    | Temperature                     | 120° F.-150° F.       |
|    | Average cathode current density | 130 a.s.f.-300 a.s.f. |

15 As previously indicated, the material advantages of the invention are obtained with a coating composed of alternate layers of two different types of chromium deposits. These advantages can be obtained with two or more layers of chromium provided that the necessary relationships between contacting chromium layers are present. In analogous arrangement, in certain instances, more than two distinctly different types of deposits may be used to obtain the unexpected benefits. The different types of deposits may be formed with different or similar 20 bath solutions. It is known that a plurality of chromium coatings having significantly different characteristics may be deposited from the same bath by adjusting the conditions of deposition. Should these latter coatings be of the required character, they may be used to practice 25 the invention.

The peculiar durability of the product of my invention appears to be associated with relative crack pattern and nobility characteristics of the chromium layers. Moreover, the relative nobility of the chromium layers to a 30 subjacent nickel layer is believed to be important to obtain optimum durability of steel parts without corrosion failure to red rust. By the use of the term "noble" or "nobility" I refer to relative differences between the electromotive potentials of two metals. A metal of 35 lesser nobility than another would be one which would exhibit an anodic potential with the other metal when the two metals comprise a voltaic cell.

40 Especially high corrosion resistance was obtained when one of the chromium layers, particularly Layer A, was 45 of a lesser nobility than the activated nickel layer. Satisfactory results may be obtained when both Layers A and B are of a lesser nobility than the activated nickel layer. However, optimum results were obtained when 50 Layer B was more noble than the nickel layer and Layer A was less noble than the nickel layer.

It is generally preferred that there be differences in the nobility of the respective chromium layers as they 55 exist in the multilayer coating. In most instances best results were obtained when these differences were approximately 0.025 volt to 0.150 volt and in certain instances differences as great as 0.175 volt may be used. Moreover, it is preferred that Layer A, when active, be 60 less noble than the nickel layer, when active. Differences in electromotive potential between these latter two layers, when activated, from about 0.025 volt to 0.10 volt and even as high as 0.13 volt are useful in obtaining the advantages of the invention.

65 Moreover, it is generally preferred that the two chromium layers of a dual chromium coating have different crack patterns. Preferably one of the layers should have a dense microscopic crack pattern while the other of the chromium layers has a comparatively sparse crack pattern. Improved results can be obtained if Layer A has a fine crack pattern and Layer B is virtually crack-free. 70 However, optimum results are obtained when the outermost chromium layer (Layer B) has the fine crack pattern and Layer A has a comparatively sparse crack pattern. Although it is preferred that Layer B have a crack pattern which is approximately 30 to 100 times denser than that of Layer A, in some instances it may be pre-

ferred to employ for Layer B a crack pattern which is only 5 times denser than that of Layer A or as much as 125 times denser than that of Layer A. Improved results may be obtained when Layer B has from about 50 to 1200 cracks per lineal inch.

Most generally I prefer to employ the more favorable relative crack pattern relationship and nobility relationship hereinafter described in combination to obtain optimum durability of the chromium plated workpiece and optimum consistency in obtaining improved durability.

Although this invention has been described in connection with certain specific examples thereof, no limitation is intended thereby except as defined in the appended claims.

I claim:

1. A method of forming a multi-layer decorative chromium coating which comprises electrodepositing a nickel coating onto the surface of a metal part, electrodepositing a first bright decorative chromium layer onto the surface of said part under an average cathode current density of approximately 90 amperes per square foot to 140 amperes per square foot from a bath at a temperature of approximately 95° F. to 115° F. containing approximately 20 ounces per gallon to 35 ounces per gallon CrO<sub>3</sub> and about .20 ounce per gallon (avdp.) to .35 ounce per gallon (avdp.) H<sub>2</sub>SO<sub>4</sub>, and then, without intervening abrasive treatment of said chromium plated surface and under an average cathode current density of approximately 130 amperes per square foot to 300 amperes per square foot, electrodepositing onto said first layer a second decorative chromium layer which has a denser crack pattern than said first layer using a bath at a temperature of approximately 120° F. to 150° F. containing about 40 ounces per gallon to 70 ounces per gallon CrO<sub>3</sub> and .45 ounce per gallon (avdp.) to .70 ounce per gallon (avdp.) H<sub>2</sub>SO<sub>4</sub>.

2. The method of forming a highly durable multi-layer decorative chromium plated article which comprises successively electrodepositing a nickel coating and two different decorative chromium layers without intervening abrasive treatment of the first chromium plated layer before application of the second chromium layer, wherein the first of said layers is electrodeposited from an aqueous bath solution which is at a temperature between 112° F. and 140° F., said bath containing less than 0.05 gram per liter of chloride ion and comprising essentially between 180 grams per liter and 540 grams per liter of CrO<sub>3</sub>, a total catalyst ion concentration of between 1.2 grams per liter and 6.3 grams per liter of sulfate and silicofluoride ions, the ratio of CrO<sub>3</sub> concentration to total catalyst ion concentration being between 20% and 85% of the total catalyst concentration, the CrO<sub>3</sub> concentration, ratio and temperature having a relationship defined by the areas enclosed by the curves in FIGURE 1 and the second of said layers is electrodeposited from an aqueous chromium plating bath containing about 100 grams to 500 grams per liter of CrO<sub>3</sub>, two catalyst-supplying compounds, and a soluble, non-catalytic compound, one of said catalyst-supplying compounds being strontium sulfate in an amount sufficient to saturate said bath and to provide an undissolved residue of strontium sulfate in the bath, the other of said catalyst-supplying compounds being an alkali metal silicofluoride in an amount sufficient to saturate said bath and to provide an undissolved residue of alkali metal silicofluoride in the bath, said alkali metal being selected from the class consisting of potassium and sodium, said non-catalytic compound being a strontium compound in an amount sufficient to suppress the concentration of said strontium sulfate in solution in said bath from the unsuppressed saturation concentration of the latter compound to a lower but greater than zero concentration.

3. The method of forming a highly durable multi-layer decorative chromium plated article which comprises successively electrodepositing a nickel coating and at least

two different decorative chromium layers without intervening abrasive treatment of the first chromium plated layer before application of the second chromium layer, wherein the first applied of said layers is electrodeposited from an aqueous bath solution which is at a temperature between 117° F. and 135° F., said bath containing less than 0.02 gram per liter of chloride ion and comprising essentially between 250 grams per liter and 425 grams per liter of CrO<sub>3</sub>, a total catalyst ion concentration of sulfate and silicofluoride ions to achieve a ratio of CrO<sub>3</sub> concentration to total catalyst ion concentration between 80:1 and 150:1, the sulfate ion content being between 35% and 75% of the total catalyst concentration, the CrO<sub>3</sub> concentration, ratio and temperature having a relationship defined by the areas enclosed by the curves in FIGURE 2 and the second applied of said layers is electrodeposited from a bath solution containing about 100 grams to 500 grams per liter of CrO<sub>3</sub>, two catalyst-supplying compounds, and a soluble, non-catalytic compound, one of said catalyst-supplying compounds being strontium sulfate in an amount sufficient to saturate said bath and to provide an undissolved residue of strontium sulfate in the bath, the other of said catalyst-supplying compounds being an alkali metal silicofluoride in an amount sufficient to saturate said bath and to provide an undissolved residue of alkali metal silicofluoride in the bath, said alkali metal being selected from the class consisting of potassium and sodium, said non-catalytic compound being a strontium compound in an amount sufficient to suppress the concentration of said strontium sulfate in solution in said bath from the unsuppressed saturation concentration of the latter compound to a lower but greater than zero concentration.

4. The method of forming a highly durable decorative chromium coating which comprises successively applying to the surface of a metal part a copper coating, a nickel coating and a multi-layer decorative chromium coating having successive layers applied without intervening abrasive treatment in which the first applied of said layers is electrodeposited from an aqueous chromium plating bath solution at a temperature between 112° F. and 140° F. said bath containing less than 0.05 gram per liter of chloride ion and comprising essentially between 180 grams per liter and 540 grams per liter of CrO<sub>3</sub>, a total catalyst ion concentration of between 1.2 grams per liter and 6.3 grams per liter of sulfate and silicofluoride ions, the ratio of CrO<sub>3</sub> concentration to total catalyst ion concentration being between 80:1 and 150:1, the sulfate ion content being between 20% and 85% of the total catalyst concentration, the CrO<sub>3</sub> concentration, ratio and temperature having a relationship defined by the areas enclosed by the curves in FIGURE 1, the sulfate in said bath being added in the form of strontium sulfate and silicofluoride added in the form of potassium silicofluoride, each in an amount sufficient to saturate said bath and to provide therein an undissolved residue of strontium sulfate and potassium silicofluoride respectively, and a soluble non-catalytic potassium compound to suppress the concentration of silicofluoride ions, the second applied of said layers being deposited from a chromium plating bath solution containing about 100 grams to 500 grams per liter of CrO<sub>3</sub>, two catalyst supplying compounds, and a soluble, non-catalytic compound, one of said catalyst-supplying compounds being strontium sulfate in an amount sufficient to saturate said bath and to provide an undissolved residue of strontium sulfate in the bath, the other of said catalyst-supplying compounds being an alkali metal silicofluoride in an amount sufficient to saturate said bath and to provide an undissolved residue of alkali metal silicofluoride in the bath, said alkali metal being selected from the class consisting of potassium and sodium, said non-catalytic compound being a strontium compound in an amount sufficient to suppress the concentration of said strontium sulfate in solution in said bath from the un-

suppressed saturation concentration of the latter compound to a lower but greater than zero concentration.

5. The method of forming a highly durable decorative chromium coating which comprises successively applying to the surface of a metal part a copper coating, a nickel coating and a multi-layer decorative chromium coating having successive layers, at least about 0.000015 inch in thickness, applied without intervening abrasive treatment in which the first applied of said layers is electrodeposited from an aqueous chromium plating bath solution at a temperature between 117° F. and 135° F., said bath containing less than 0.02 gram per liter of chloride ion and comprising essentially between 250 grams per liter and 425 grams per liter of CrO<sub>3</sub>, a total catalyst ion concentration of sulfate and silicofluoride ions to achieve a ratio of CrO<sub>3</sub> concentration to total catalyst ion concentration between 80:1 and 150:1, the sulfate ion content being between 35% and 75% of the total catalyst concentration, the CrO<sub>3</sub> concentration, ratio and temperature having a relationship defined by the areas enclosed by the curves in FIGURE 2, and the second applied of said layers being deposited from an aqueous bath solution containing about 100 grams to 500 grams per liter of CrO<sub>3</sub>, two catalyst supplying compounds, and a soluble, non-catalytic compound, one of said catalyst-supplying compounds being strontium sulfate in an amount sufficient to saturate said bath and to provide an undissolved residue of strontium sulfate in the bath, the other of said catalyst-supplying compounds being an alkali metal silicofluoride in an amount sufficient to saturate said bath and

5

10

to provide an undissolved residue of alkali metal silicofluoride in the bath, said alkali metal being selected from the class consisting of potassium and sodium, said non-catalytic compound being a strontium compound in an amount sufficient to suppress the concentration of said strontium sulfate in solution in said bath from the unsuppressed saturation concentration of the latter compound to a lower but greater than zero concentration.

## References Cited in the file of this patent

## UNITED STATES PATENTS

|           |             |                |
|-----------|-------------|----------------|
| 1,746,751 | Van Derhoef | Feb. 11, 1930  |
| 1,813,842 | Fink        | July 7, 1931   |
| 1,836,598 | Humphries   | Dec. 15, 1931  |
| 2,018,814 | Smith       | Oct. 29, 1935  |
| 2,093,428 | Ford        | Sept. 21, 1937 |
| 2,412,977 | Eskin       | Dec. 24, 1946  |
| 2,640,022 | Stareck     | May 26, 1953   |
| 2,678,908 | Tucker      | May 8, 1954    |
| 2,800,437 | Stareck     | July 23, 1957  |
| 2,800,438 | Stareck     | July 23, 1957  |
| 2,822,326 | Safranek    | Feb. 4, 1958   |
| 2,856,334 | Topelain    | Oct. 14, 1958  |
| 2,898,234 | Nack        | Aug. 4, 1959   |
| 2,916,424 | Stareck     | Dec. 8, 1959   |
| 2,952,590 | Stareck     | Sept. 13, 1960 |

30 568,161

## FOREIGN PATENTS

Great Britain ----- Mar. 21, 1945

UNITED STATES PATENT OFFICE  
CERTIFICATE OF CORRECTION

Patent No. 3,157,585

November 17, 1964

Rollie P. Durham

It is hereby certified that error appears in the above numbered patent requiring correction and that the said Letters Patent should read as corrected below.

Column 2, line 2, for "aoid" read -- acid --; line 35, for "(hydrate)" read -- (hydrated) --; column 4, line 56, for "abtain" read -- obtain --; line 62, for "centration" read -- concentration --; line 71, for "may" read -- my --.

Signed and sealed this 6th day of April 1965.

(SEAL)

Attest:

ERNEST W. SWIDER  
Attesting Officer

EDWARD J. BRENNER  
Commissioner of Patents